



US007362209B2

(12) **United States Patent**  
**Ohashi et al.**

(10) **Patent No.:** **US 7,362,209 B2**  
(45) **Date of Patent:** **Apr. 22, 2008**

- (54) **ZINC OXIDE RESISTOR AND ITS MANUFACTURING METHOD**
- (75) Inventors: **Naoki Ohashi**, Ibaraki (JP); **Hajime Haneda**, Ibaraki (JP); **Isao Sakaguchi**, Ibaraki (JP); **Takeshi Ohgaki**, Ibaraki (JP); **Ken Kataoka**, Ibaraki (JP)
- (73) Assignee: **National Institute for Materials Science**, Tsukuba-shi (JP)
- (\*) Notice: Subject to any disclaimer, the term of this patent is extended or adjusted under 35 U.S.C. 154(b) by 260 days.
- (21) Appl. No.: **10/537,492**
- (22) PCT Filed: **Dec. 2, 2003**
- (86) PCT No.: **PCT/JP03/15448**
- § 371 (c)(1),  
(2), (4) Date: **Dec. 14, 2005**
- (87) PCT Pub. No.: **WO2004/051676**
- PCT Pub. Date: **Jun. 17, 2004**
- (65) **Prior Publication Data**  
US 2006/0164200 A1 Jul. 27, 2006
- (30) **Foreign Application Priority Data**  
Dec. 3, 2002 (JP) ..... 2002-350574
- (51) **Int. Cl.**  
**H01C 7/10** (2006.01)  
**H01C 7/13** (2006.01)
- (52) **U.S. Cl.** ..... **338/20**; 338/22 R; 252/518;  
252/521
- (58) **Field of Classification Search** ..... 338/20-25;  
29/610 R; 252/518, 521, 500, 519.5, 519.51,  
252/520.52

See application file for complete search history.

- (56) **References Cited**
- U.S. PATENT DOCUMENTS
- 4,420,737 A \* 12/1983 Miyoshi et al. ..... 338/21
- (Continued)
- FOREIGN PATENT DOCUMENTS
- JP 2-219203 8/1990
- (Continued)
- OTHER PUBLICATIONS
- M. Matsuoka, *Nonohmic Properties of Zinc Oxide Ceramics*, Japanese Journal of Applied Physics, vol. 10, No. 6, Jun. 1971, pp. 736-746.

(Continued)

Primary Examiner—K. Richard Lee  
(74) Attorney, Agent, or Firm—Westerman, Hattori, Daniels & Adrian, LLP.

(57) **ABSTRACT**

Disclosed are a zinc oxide resistor structure, and methods of forming a glass layer and a resistor, which are required for producing the resistor structure. The zinc oxide resistor comprises zinc oxide grains and an oxide glass layer which contains bismuth and boron and intervenes between the zinc oxide grains. The oxide glass layer residing between the zinc oxide grains changes the electric properties between the grains to achieve a higher resistance and a non-ohmic characteristic of a voltage-dependent resistance value in the resistor. This non-ohmic characteristic can be applied, particularly, to a non-ohmic device to be compatible with a low-voltage operation. Differently from conventional resistors, the oxide glass layer intervening between the zinc oxide grains can achieve an enhanced mechanical strength of a junction in the device.

**12 Claims, 6 Drawing Sheets**



U.S. PATENT DOCUMENTS

4,959,262 A \* 9/1990 Charles et al. .... 428/329  
5,770,113 A \* 6/1998 Iga et al. .... 252/519.51  
6,184,771 B1 \* 2/2001 Suzuki et al. .... 338/21

FOREIGN PATENT DOCUMENTS

JP 10-270214 A 10/1998  
JP 2000-228302 8/2000

OTHER PUBLICATIONS

A. Tanaka et al., *Evaluation of Single Grain Boundaries in ZnO: Rare-Earth Varistor by Micro-Electrodes*, Key Engineering Mate-

rials, vol. 157-158, CSJ Series—Publications of the Ceramic Society of Japan, vol. 1, 1999, pp. 235-240.

U. Schwing et al., *Model experiments describing the microcontact of ZnO varistors*, Journal of Applied Physics, 57(12), Jun. 15, 1985, pp. 5372-5379.

N. Ohashi et al., *Synthesis of ZnO Bicrystals Doped with Co or Mn and Their Electrical Properties*, Japanese Journal of Applied Physics, vol. 38, Part 1, No. 9A, Sep. 1999, pp. 5028-5032.

Y. Sato et al., *Current-Voltage Characteristics across [0001]Twist Boundaries in Zinc Oxide Bicrystals*, Journal of the American Ceramic Society, 85 (8), Aug. 2002, pp. 2142-2144.

\* cited by examiner

FIG.1



FIG.2



FIG.3



FIG.4



FIG.5



FIG.6



FIG.7



FIG.8(A)



FIG.8(B)



# ZINC OXIDE RESISTOR AND ITS MANUFACTURING METHOD

## TECHNICAL FIELD

The present invention relates to a zinc oxide resistor, and more particularly a varistor device structure for protecting an electric/electronic circuit from surge voltages, and a production method thereof.

## BACKGROUND ART

### 1. Typical Zinc Oxide Varsity

Generally, a zinc oxide varistor is provided as a polycrystalline zinc-oxide ceramics. Specifically, the zinc oxide varistor has been produced by mixing zinc oxide powder, transition metal oxide powder and bismuth oxide powder, and burning the mixture at a high temperature, to form a polycrystalline body with a structure in which a bismuth oxide or the like is segregated in the boundaries between zinc oxide grains each containing a transition metal oxide dissolved therein in the form of a solid solution (see, for example, the following Non-Patent Publication 1).

An appropriate additive makes it possible for the zinc oxide ceramics to exhibit a nonlinear current-voltage characteristic in which each grain boundary in the zinc oxide ceramics has an operating voltage of about 3 V (see, for example, the following Non-Patent Publication 2). That is, the operating voltage as one of varistor characteristics is generally determined by the number of grain boundaries. Specifically, as shown in FIG. 7, in a varistor device comprising two electrodes 2A, 2B provided at opposite end surfaces thereof and zinc oxide (ZnO) grains 1 residing therebetween, an overall operating voltage of the varistor device is determined by the product of the number of boundaries between the zinc oxide grains 1 and the operating voltage having the nonlinear current-voltage characteristic in each of the grain boundaries. Thus, the size of the zinc oxide grains 1 in the zinc oxide ceramics inherently contributes to the varistor characteristics.

The grain size of a ceramics depends on an additive and a burning temperature, and generally has a statistical distribution. This causes difficulties in setting the number of grains or each size of grains in a ceramics at a predetermined value. Therefore, the production of a low-voltage type varistor essentially requires a particular technique in addition to a simple burning technique for forming a ceramics. For example, a varistor device having an operating voltage of 30 KV is required to ensure 10000 grain boundaries each having an operating voltage of 3 V. In contrast, a varistor device having an operating voltage of 6 V means a ceramics which includes 2 grain boundaries each having an operating voltage of 3 V, or only 3 grains. That is, some technique for forming a ceramics having a small number of grain boundaries is required to produce a varistor operable at a low voltage.

### 2. Multilayer Varsity

As one technique for producing a varistor having a small number of grain boundaries, or a low operating voltage, there has been known multilayering (see, for example, the following Patent Publication 1). This technique comprises preparing a sheet-shaped compact to be burned as a ceramics, and forming alternate layers of a metal electrode layer and a zinc-oxide ceramics layer, as shown in FIG. 8(A). The intervening metal layer makes it possible to hinder the

contact between the zinc oxide grains or reduce the number of grain boundaries so as to achieve a varistor having a low operating voltage.

However, as seen in the enlarged view of FIG. 8(A), while each of a grain boundary 1 and a grain boundary 2 of the ZnO grains 1 extending in a direction orthogonal to a current path contributes to varistor characteristics, a grain boundary 3 extending parallel to a current path would be unnecessary in view of enhancement of varistor characteristics. Moreover, a current flowing along a current path P1 comes across three grain boundaries, and a current flowing along a current path P2 comes across four grain boundaries. This means that an operating voltage of the varistor differs between the current paths P1, P2. Thus, a varistor operation at lower voltage can be achieved only if the number of grain boundaries is more strictly controlled.

### 3. Single-Grain-Boundary Varsity

It is known that each grain boundary of a zinc oxide varistor containing an appropriate additive has an operating voltage of 3 V. Thus, a low-voltage type varistor having any operating voltage of an integral multiple of 3 V can be produced by preparing a plurality of varistors each with a single grain boundary, and connecting them in series.

There has been known a single-grain-boundary varistor 25 experimentally produced by forming a bismuth-containing oxide crystal phase intervening between zinc-oxide single crystals (see, for example, the following Non-Patent Publication 3). While this technique can achieve a current-voltage characteristic with high nonlinearity, it still involves a problem about strength of a junction between the opposed zinc-oxide single crystals. The single-grain-boundary varistor produced through a process utilizing a crystalline grain-boundary layer as disclosed in the Non-Patent Publication 3 leaves a problem about mechanical strength of a junction 30 therein, as in the after-mentioned Comparative Examples.

There has also been known a single-grain-boundary varistor device obtained by fundamentally joining zinc-oxide single crystals together without forming an intervening crystal phase between grain boundaries (see, for example, 40 the following Non-Patent Publications 4 and 5). While a certain level of mechanical strength is achieved in the varistor device disclosed in the Non-Patent Publication 4, the varistor device without any intervening grain-boundary layer has a poor performance, wherein an  $\alpha$ -value as a 45 performance index of varistor characteristics is less than 10. Similarly, adequate varistor characteristics are not achieved in the varistor device disclosed in the Non-Patent Publication 5, due to no intervening grain-boundary layer. However, the Non-Patent Publications 4 includes a valuable suggestion that, while a nonlinear current-voltage characteristic is 50 achieved by joining zinc-oxide single crystals each containing manganese and cobalt dissolved therein in the form of a solid solution, no nonlinear current-voltage characteristic is achieved if single crystals without addition of manganese and cobalt are joined together.

[Patent Publication 1] Japanese Patent Laid-Open Publication No. 10-270214

[Non-Patent Publication 1] M. Matsuoka, Jpn. J. Appl. Phys. 10, 736-746 (1071)

[Non-Patent Publication 2] "Evaluation of Single Grain Boundaries in ZnO: Rare-Earth Varsity by Micro-Electrodes" S. Tanaka, K. Takahashi; "Key Engineering Materials Series, Vol. 157-158, CSJ Series Vol. 1, (Electroceramics in Japan I)" p 241 (1998), (Trans Tech Publication, 60 Switzerland)

[Non-Patent Publication 3] "MODEL EXPERIMENTS DESCRIBING THE MICRO-CONTACT OF ZnO VARIS-

TORS", SCHWINGU, HOFFMANN B, JOURNAL OF APPLIED PHYSICS, 57 (12): 5372-5379 (1985)

[Non-Patent Publication 4] "Synthesis of ZnO bicrystals doped with Co or Mn and their electrical properties" Ohashi N, Terada Y, Ohgaki T, Tanaka S, Turumi T, Fukunaga O, Haneda H, Tanaka J, JAPANESE JOURNAL OF APPLIED PHYSICS PART 1-REGULAR PAPER SHORT NOTES & REVIEW PAPERS, 38 (9A): 5028-5032, SEPTEMBER (1999)

[Non-Patent Publication 5] "Current-voltage characteristic across [0001] twist boundaries in zinc oxide bicrystals" Sato Y, Oba F, Yamamoto T, Ikuhashi Y, Sakuma T, JOURNAL OF THE AMERICAN CERAMIC SOCIETY, 85 (8): 2142-2144, AUGUST (2002)

### DISCLOSURE OF INVENTION

In view of the above circumstances, it is an object of the present invention to provide a single-grain-boundary varistor device or a zinc oxide resistor exhibiting varistor characteristics based on an artificial grain boundary obtained by joining zinc-oxide single crystals.

It is another object of the present invention to provide a zinc oxide resistor structure capable of achieving an  $\alpha$ -value, or a performance index of a zinc oxide varistor, of about 20 or more, which is equivalent to that of a conventional typical polycrystalline varistor device, and joining zinc-oxide single crystals with a high junction strength in an obtained artificial grain boundary, so as to eliminate the risk of peeling of the zinc-oxide single crystals during use.

It is yet another object of the present invention to provide a method of producing such a zinc oxide resistor.

The present invention provides a zinc oxide varistor having varistor characteristics achieved by a structure which comprises a pair of opposed zinc-oxide single crystals each containing cobalt and manganese dissolved therein in the form of a solid solution, and a glass layer forming an oxide grain boundary layer which includes a primary component consisting of bismuth and boron and intervenes between the zinc-oxide single crystals.

The present invention provides a structure and production method for achieving zinc oxide varistor characteristics conventionally achieved in a zinc oxide sintered body, by a multilayer comprising a pair of opposed single crystals and a glass layer forming an oxide grain boundary layer. Thus, differently from a conventional varistor consisting of polycrystalline body, the technique of joining the opposed single crystals makes it possible to provide enhanced controllability of a resistor so as to obtain a varistor having an intended function.

In order to achieve the above objects, the following techniques are employed.

(A) Use of Zinc-Oxide Single Crystals each containing Cobalt and Manganese

A pair of zinc-oxide single crystals containing cobalt and manganese dissolved therein in the form of a solid solution are joined together to form a joined unit so as to provide a nonlinear current-voltage characteristic in a resistor having the joined zinc-oxide single crystals.

(B) Presence of Grain Boundary Layer containing Bismuth Oxide

Instead of simply joining the zinc-oxide single crystals, an intervening layer containing bismuth oxide is formed in the junction interface between the zinc-oxide single crystals to enhance the nonlinear current-voltage characteristic of the zinc oxide varistor.

(C) Non-Crystallization of Grain Boundary Layer containing Bismuth Oxide

If the bismuth oxide layer intervening between the grain boundaries in the joined unit of the zinc-oxide single crystals is crystallized, the mechanical strength of the joined unit is likely to be spoiled, as described above. Thus, the grain boundary layer of the joined unit is formed of a bismuth- and-boron-containing oxide glass phase. In a process of forming this glass phase, the boron oxide added to the bismuth-containing layer residing in the junction interface can accelerate vitrification of the grain boundary layer by taking advantage of its feature of a low melting point.

The zinc-oxide varistor or resistor has a current-voltage characteristic with significantly high nonlinearity, and a resistance value to be reduced in response to a high-voltage noise. Based on these features, the zinc-oxide resistor is used for protecting an electric/electronic circuit from an abnormal high voltage. The junction interface between the zinc-oxide single crystal/grain boundary layer/zinc-oxide single crystal 15 20 25 30 35 40 45 50 55 60 65 70 75 80 85 90 95 100 single crystal/grain boundary layer/zinc-oxide single crystal 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9

FIG. 6 is a graph showing a current-voltage characteristic at room temperature of a zinc oxide resistor obtained in Inventive Example 2.

FIG. 7 is a schematic diagram of a conventional zinc oxide varistor.

FIG. 8 is a schematic diagram of a conventional multi-layer zinc oxide varistor.

#### BEST MODE FOR CARRYING OUT THE INVENTION

(1) A zinc oxide resistor of the present invention provides comprises as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals. The zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein.

FIG. 1 shows a nonlinear resistor which has the so-called "varistor characteristics", and a structure with only one grain boundary formed by joining a pair of opposed single crystals. Specifically, the grain boundary is formed by disposing a pair of zinc-oxide single crystals 1A, 1B each containing cobalt and manganese dissolved therein in the form of a solid solution, in opposed relation to one another between a pair of electrodes 2A, 2B. The cobalt and manganese are elements which are considered to be essential to the expression of nonlinearity, as disclosed in the aforementioned Non-Patent Publication 4.

As disclosed in the Non-Patent Publication 3, the nonlinearity can be enhanced by segregating a grain boundary layer containing bismuth, in the grain boundary. Thus, an oxide layer 3 containing bismuth is provided as an interface layer disposed between the zinc-oxide single crystals 1A, 1B. Additionally, in order to ensure a sufficient mechanical strength in the junction between the opposed zinc-oxide single crystals 1A, 1B or prevent the peeling of the opposed zinc-oxide single crystals 1A, 1B, the oxide layer 3 is formed as a glass phase containing bismuth oxide and boron oxide to provide enhanced junction strength.

When a zinc-oxide based nonlinear resistor is produced by the addition of bismuth, cobalt and manganese, an auxiliary additive, such as antimony, may be added to provide enhanced characteristics, as is generally known. While cobalt, manganese, bismuth and boron are used as additives in the zinc-oxide resistor structure of the present invention, it is to be understood that any other suitable auxiliary additive may be additionally used. The essence of the present invention lies in forming the bismuth-and-boron-containing oxide glass phase in the junction between the opposed zinc-oxide single crystals. Thus, it is not essential to the present invention whether an auxiliary additive other than cobalt and manganese is added to the opposed zinc-oxide single crystals.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide

which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (2) each of the opposed zinc-oxide single crystals may contain the cobalt dissolved therein in the form of a solid solution, in an amount of 0.5 mol % or more with respect to zinc therein.

As described above, cobalt is one essential element to the expression of nonlinearity. When it is necessary to achieve high nonlinearity in the zinc oxide resistor of the present invention having the interface layer formed as a glass phase containing a primary component consisting of bismuth and boron, each of the opposed zinc-oxide single crystals preferably contains the cobalt dissolved therein in the form of a solid solution, in an amount of 0.5 mol % or more. In an actual production process for the resistor, it is desirable that an optimal cobalt concentration for achieving intended resistor characteristics is experimentally determined while taking account of the type and concentration of each impurity originally contained in zinc-oxide single crystals to be used. In this case, the solid solubility of cobalt into zinc oxide has a given limit, and the upper limit is determined by the solid solubility of the cobalt in the zinc oxide.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (3) each of the opposed zinc-oxide single crystals may contain the manganese dissolved therein in the form of a solid solution, in an amount of 0.05 mol % or more with respect to zinc therein.

The addition of manganese can bring about an effect of reducing a leak current due to the grain boundary to provide enhanced nonlinearity.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (4) each of the opposed zinc-oxide single crystals may have a length of 5 mm, a width of 5 mm, and a thickness of 0.5 mm, and the oxide containing a primary component consisting of bismuth and boron, to be used for forming a junction between the opposed zinc-oxide single crystals, may be a glass prepared in such a manner as to contain, in oxide wt %

equivalent, 37.0 to 22.7 wt % of  $B_2O_3$ , 3.8 to 1.9 wt % of  $Co_2O_3$  and 5.7 to 1.6 wt % of  $MnO_2$ , with the remainder being bismuth oxide.

The above composition of the interface layer is effective in producing the zinc oxide resistor using zinc-oxide single crystals prepared by cutting a commercially-available zinc-oxide single crystal having a typical thickness of 0.5 mm, into a size of 5×5 mm, to achieve excellent junction and nonlinearity. The present invention is not limited to the above composition, but any other suitable composition may be appropriately selected depending on the thickness of each zinc-oxide single crystal to be used, the type and quantity of element originally dissolved in the zinc-oxide single crystals to be joined, in the form of a solid solution, resistance characteristics required for the joined unit, and other factors. In the same manner, a temperature and/or time-period in the process of forming the junction may also be appropriately selected.

The above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (5) may exhibit an  $\alpha$ -value of 20 or more, as a performance index of a zinc oxide varistor.

Specifically, the zinc oxide resistor has the opposed zinc-oxide single crystals containing the cobalt and manganese dissolved therein in a solid solution, and the grain boundary layer having the bismuth-and-boron-containing oxide glass phase and intervening in the joined unit. Particularly, based on this structure, the zinc oxide resistor exhibits an  $\alpha$ -value of 20 or more, as a performance index of a zinc oxide varistor.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (6) the (zinc-oxide single crystal/bismuth-boron based oxide interface layer/zinc-oxide single crystal) structure serving as the basic unit may have an operating voltage of  $2.9 \pm 0.3$  V, as a performance index of a zinc oxide varistor.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth

and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (7) the (zinc-oxide single crystal/bismuth-boron based oxide interface layer/zinc-oxide single crystal) structure may be provided in a number of n. In this case, the structures of the number n may be repeatedly superimposed in a layered manner, and provided with a zinc-oxide single crystal superimposed thereon to form a (n+1) layered structure including the number (n+1) of zinc-oxide single crystals and the number n of bismuth-boron based oxide interface layers. The zinc-oxide resistor has an operating voltage of  $(2.9 \pm 0.3) n$  V, as a performance index of a zinc oxide varistor.

Specifically, the operating voltage of  $2.9 \pm 0.3$  V is achieved by a single junction, and the structures of the number n can be superimposed in a layered manner as shown in FIG. 2 to provide a multilayer zinc oxide resistor having any desired operating voltage.

In the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, (8) the (zinc-oxide single crystal/bismuth-boron based oxide interface layer/zinc-oxide single crystal) structure may be adjusted to have an operating voltage of x V, as a performance index of a zinc oxide varistor, and provided in a number of n. In this case, the structures of number n may be electrically connected in series. The zinc-oxide resistor has an operation voltage of  $n \times x$  V, as a performance index of a zinc oxide varistor.

Specifically, the operating voltage of  $2.9 \pm 0.3$  V is achieved by a single junction, and the structures of the number n can be electrically connected to each other using lead wires as shown in FIG. 3 to provide a series-connected zinc oxide resistor having any desired operating voltage.

(9) A method of producing either one of the above zinc oxide resistors (1) to (7) of the present invention, comprises: disposing an oxide containing bismuth and boron, between a pair of opposed zinc-oxide single crystals to form a sandwich structure of (a zinc-oxide single crystal/a composition to be formed as a glass phase/a zinc-oxide single crystal); heating and holding the sandwich structure at a high temperature allowing the oxide containing bismuth and boron, to be molten; and rapidly cooling the heated sandwich structure to join the pair of zinc-oxide single crystals with a glass-phase oxide interface layer intervening therebetween.

In this method, a process of disposing the bismuth-and-boron-containing oxide between the opposed zinc-oxide single crystals, to form the sandwich structure of (a zinc-oxide single crystal/a composition to be formed as a glass phase/a zinc-oxide single crystal), includes a plurality of options. FIG. 4 shows this process. In one of the options, a suitable material for forming a desired glass phase is molten

and vitrified in advance using a crucible, such as a platinum crucible, and then crushed to obtain a glass powder. In another option, a composition to be formed as a desired glass phase is placed on one zinc-oxide single crystal to be joined, and the zinc-oxide single crystal is used as a plate for vitrification without using a crucible. In the former case, the obtained glass phase is disposed between a pair of zinc-oxide single crystals to be joined, and then they are subjected to a heat treatment to form a junction between the zinc-oxide single crystals. In the latter case, another zinc-oxide single crystal is disposed in opposed relation to the zinc-oxide single crystal having the vitrified composition attached thereon, and they are subjected to a heat treatment to form a junction between the zinc-oxide single crystals.

In this process, a time-period of the heat treatment for heating the sandwich structure at a high temperature to melt the glass and form the junction is not limited to a specific value. While the heat-treatment time is required to set at a sufficient value for allowing the glass to be homogenized, an excessive heat-treatment time induces a reaction between the glass components and the zinc-oxide single crystals to cause elution of zinc oxide into the glass components. Thus, it is practically desirable to prepare a glass powder in advance as in the former case, and, after heating the glass powder at a high temperature allowing the glass to be molten, for a melting time of about 3 to 12 hours, rapidly cool the glass.

In either case, it is desirable to optimize the composition of the glass phase in consideration of wettability to zinc oxide so as to obtain the aforementioned required structure of the zinc oxide resistor. For example, the glass composition is preferably determined by synthesizing a glass phase containing bismuth and boron, melting and rapidly cooling the glass on the zinc-oxide single crystal to form a joined unit of zinc oxide and glass droplets, calculating a contact angle between the glass and the zinc-oxide single crystal based on this joined unit, selecting a glass allowing the contact angle to be 5 degrees or less.

In the above production method, it is not specified whether cobalt and manganese are added to the glass. If each of the zinc-oxide single crystals to be joined has a thin-plate shape, cobalt and manganese may be added in advance to glass components to be formed as the grain boundary of the joined unit, and diffused in the zinc-oxide single crystals in conjunction with the process of subjecting the sandwich structure to a heat treatment at a high temperature to melt the glass and form the junction.

If each of the zinc-oxide single crystals to be joined has a thick-plate shape, the heat treatment time for forming the junction is likely to cause insufficient diffusion of the cobalt and manganese from the molten glass to the zinc oxide. Thus, irrelevant to each thickness of the zinc-oxide single crystals, the above production method is preferably implemented in such a manner that a pair of zinc-oxide single crystals each containing cobalt and manganese diffused therein in advance is used together with the glass components to form the sandwich structure, and then the sandwich structure is subjected to a heat treatment at a high temperature to form the junction.

The above production method is only one typical example. Thus, any other suitable method may be used to produce the above zinc oxide resistor comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a

primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein. That is, the above zinc oxide resistor of the present invention comprising as a basic unit a structure of (a zinc-oxide single crystal/a bismuth-boron based oxide interface layer/a zinc-oxide single crystal) formed of a pair of opposed zinc-oxide single crystals each containing cobalt and manganese dissolved therein in the form of a solid solution, and an oxide which contains a primary component consisting of bismuth and boron and intervenes between the zinc-oxide single crystals, wherein the zinc oxide resistor has non-ohmic properties or exhibits zinc-oxide varistor characteristics, based on the intervening oxide interface layer, and the bismuth-boron based oxide interface layer is formed as a bismuth-and-boron-containing oxide glass phase by the action of the boron contained therein, is not limited by a production method thereof.

(10) A method of producing either one of the above zinc oxide resistors (1) to (7) of the present invention, comprises: bringing each of two zinc-oxide single crystals into contact with a chunk of oxide cobalt, and heating the zinc-oxide single crystals and the chunk of oxide cobalt at a high temperature capable of inducing a diffusion reaction to diffuse cobalt from the chunk of oxide cobalt into the zinc-oxide single crystals so as to prepare a pair of zinc-oxide single crystals in such a manner as to have a cobalt concentration of 0.5 mol % or more; disposing an oxide containing bismuth and boron, between the pair of zinc-oxide single crystals disposed opposed to one another, to form a sandwich structure of (a zinc-oxide single crystal/a composition to be formed as a glass phase/a zinc-oxide single crystal); heating and holding the sandwich structure at a high temperature allowing the bismuth-and-boron-containing oxide to be molten; and rapidly cooling the heated sandwich structure to join the pair of zinc-oxide single crystals with a glass-phase oxide interface layer intervening therebetween.

Specifically, in order to obtain enhanced characteristics in the zinc oxide resistor through the production method of the present invention, it is required to adjust the concentration of cobalt in the zinc-oxide single crystals to be joined, at a desired value. Thus, if a commercially-available zinc-oxide single crystal containing no cobalt, it is necessary to introduce an appropriate amount of cobalt into the single crystal. In this process of introducing cobalt, it is desirable to introduce a high concentration of cobalt without roughening the surface of the zinc-oxide single crystal.

For this purpose, cobalt can be conveniently introduced into a zinc-oxide single crystal by preparing a chunk containing a primary component consisting of oxide cobalt, bringing the chunk of oxide cobalt into contact with a target zinc-oxide single crystal, and heating and holding them at a high temperature. A measurement based on light absorption spectrum may be conveniently used for determining a quantity of cobalt to be introduced, in a nondestructive manner. In this case, an analytical curve may be made in advance to calculate a quantity of cobalt to be added, based on light absorption spectrum.

(11) In the production method (9) or (10) of the present invention, when each of the opposed zinc-oxide single crystals has a length of 5 mm, a width of 5 mm, and a thickness of 0.5 mm, the oxide containing a primary com-

## 11

ponent consisting of bismuth and boron, to be used for forming a junction between the opposed zinc-oxide single crystals, may be a glass prepared in such a manner as to contain, in oxide wt % equivalent, 37.0 to 22.7 wt % of  $B_2O_3$ , 3.8 to 1.9 wt % of  $Co_2O_3$  and 5.7 to 1.6 wt % of  $MnO_2$ , with the remainder being bismuth oxide.

Specifically, each optimal quantity of cobalt, manganese, bismuth and boron to be contained in the glass phase differs depending on each size of the opposed zinc-oxide single crystals to be joined, and the type and quantity of additives originally containing therein. Thus, the above composition is simply shown as one example capable of producing a nonlinear resistor using the zinc-oxide single crystals each having a length of 5 mm, a width of 5 mm, and a thickness of 0.5 mm. Therefore, the above composition is not always an applicable value to all of zinc oxide resistors having the interface layer formed as a bismuth-and-boron-containing oxide glass phase according to the present invention.

(12) In either one of the production methods (9) to (11) of the present invention, the oxide containing a primary component consisting of bismuth and boron, to be used for forming a junction between the opposed zinc-oxide single crystals, may be a glass. In this case, the method may include flattening each surface of the opposed zinc-oxide single crystals through mirror polishing, and adjusting a quantity of the glass in such a manner that a molar ratio of the glass quantity in an equivalent bismuth quantity contained in the glass to a quantity of the opposed zinc-oxide single crystals, is set at 1.2 mol %.

This total quantity of the glass phase for forming the junction simply shows a desirable value in one case where each surface of the opposed zinc-oxide single crystals is flattened through mirror polishing. Fundamentally, it is desirable that the total quantity of the glass phase for forming the junction is optimized in consideration of each flatness or surface area of the opposed zinc-oxide single crystals to be joined. Thus, in advance of an actual production, it is desirable to determine an optimal amount of bismuth with reference to the above recommended value.

## EXAMPLE

## Inventive Example 1

Each of two zinc-oxide single crystals was in contact with a cobalt-oxide sintered body, in an oxygen flow at 1200° C. for 3 hours to diffuse cobalt into each zinc-oxide single crystal so as to prepare two cobalt-doped zinc-oxide single crystals. A quantity of the resulting solid solution of cobalt was calculated as about 1 at % based on optical spectrum. Then, 0.8772 g of boron oxide, 8.8068 g of bismuth oxide, 0.1517 g of cobalt oxide and 0.16431 g of manganese oxide were measured and mixed together. The obtained mixture was put in a platinum crucible, and molten at 900° C. in an oxygen flow. Then, the molten mixture was flowed out of the crucible, and solidified to obtain a bismuth-and-boron-containing oxide glass. After crushing the glass, the obtained glass powder was dredged on one of the prepared cobalt-doped zinc-oxide single crystals (5×5×0.5 mm), and another zinc-oxide single crystal was superimposed on the single crystal with the glass powder to form a sandwich structure.

Without particular pressing, the sandwich structure was heated at 1000° C. in an oxygen flow for 12 hours, and then cooled to room temperature over a period of about 5 hours to produce a zinc oxide resistor. The manganese was dissolved in the zinc-oxide single crystals through diffusion. As

## 12

shown in FIG. 5, the obtained zinc oxide resistor exhibited a current-voltage characteristic represented by  $\alpha=20$ .

## Inventive Example 2

Each of two zinc-oxide single crystals was in contact with a cobalt-oxide sintered body, in an oxygen flow at 1200° C. for 12 hours to diffuse cobalt into each zinc-oxide single crystal so as to prepare two cobalt-doped zinc-oxide single crystals. Then, 0.8772 g of boron oxide, 8.8068 g of bismuth oxide, 0.1517 g of cobalt oxide and 0.16431 g of manganese oxide were measured and mixed together. The obtained mixture was put in a platinum crucible, and molten at 900° C. in an oxygen flow. Then, the molten mixture was flowed out of the crucible, and solidified to obtain a bismuth-and-boron-containing oxide glass. After crushing the glass, the obtained glass powder was dredged on one of the prepared cobalt-doped zinc-oxide single crystals (5×5×0.5 mm), and another zinc-oxide single crystal was superimposed on the single crystal with the glass powder to form a sandwich structure.

Without particular pressing, the sandwich structure was heated at 1000° C. in an oxygen flow for 4 hours, and then cooled to room temperature over a period of about 5 hours to produce a zinc oxide resistor. The manganese was dissolved in the zinc-oxide single crystals through diffusion. As shown in FIG. 6, the obtained zinc oxide resistor exhibited a current-voltage characteristic represented by  $\alpha=26$ .

## Comparative Example 1

9.5762 g of bismuth oxide, 0.2749 g of cobalt oxide and 0.1489 g of manganese oxide were measured and mixed together. The obtained mixture was put in a platinum crucible, and molten at 900° C. in an oxygen flow. Then, the molten mixture was flowed out of the crucible, and solidified to obtain a bismuth-containing oxide glass without boron. Through x-ray diffraction measurement, it was proven that the obtained oxide is a crystal phase. After crushing the bismuth-containing oxide glass, the obtained glass powder was dredged on one of two cobalt-doped zinc-oxide single crystals (5×5×0.5 mm) prepared in advance, and another zinc-oxide single crystal was superimposed on the single crystal with the glass powder to form a sandwich structure.

Without particular pressing, the sandwich structure was heated at 1000° C. in an oxygen flow for 1 hour, and then cooled to room temperature over a period of about 5 hours to produce a zinc oxide resistor. While a measurement about characteristics was attempted in the same manner as that in Incentive Examples 1 and 2, the zinc-oxide single crystals was peeled from one another during the measurement due to poor junction strength. The reason would be that the interface layer is formed as polycrystal due to no addition of boron into the interface layer, and consequently grain boundaries and/or cracks are formed in the interface layer to cause deterioration in mechanical strength.

## Comparative Example 2

0.6018 g of boron oxide and 9.3982 g of bismuth oxide were measured and mixed together. The obtained mixture was put in a platinum crucible, and molten at 900° C. in an oxygen flow. Then, the molten mixture was flowed out of the crucible, and solidified to obtain a bismuth-and-boron-containing oxide glass. After crushing the bismuth-and-boron-containing oxide glass, the obtained glass powder was dredged on one of two cobalt-doped zinc-oxide single

## 13

crystals (5×5×0.5 mm) prepared in advance without a cobalt diffusion treatment, and another zinc-oxide single crystal was superimposed on the single crystal with the glass powder to form a sandwich structure.

Without particular pressing, the sandwich structure was heated at 1000° C. in an oxygen flow for 4 hours, and then cooled to room temperature over a period of about 5 hours to produce a zinc oxide resistor. While a measurement about characteristics was attempted in the same manner as that in Incentive Examples 1 and 2, a linear current-voltage characteristic was obtained without any observation of a non-linear current-voltage characteristic

## INDUSTRIAL APPLICABILITY

Differently from a high-voltage varistor as typified by arrestors, the zinc oxide resistor of the present invention is applicable to a low-voltage varistor, and usable in removing low-voltage noises in electronic components.

What is claimed is:

1. A zinc oxide resistor comprising:  
a pair of opposed zinc-oxide single crystals each containing cobalt and manganese dissolved therein in the form of a solid solution, and  
a bismuth-boron based oxide interface layer intervening between said zinc-oxide single crystals,  
wherein said zinc oxide resistor has non-ohmic properties or exhibits zinc-oxide varistor characteristics, and said bismuth-boron based oxide interface layer includes a bismuth-and-boron-containing oxide glass phase.
2. The zinc oxide resistor as defined in claim 1, wherein each of said opposed zinc-oxide single crystals contains said cobalt dissolved therein in the form of a solid solution, in an amount of 0.5 mol % or more with respect to zinc therein.
3. The zinc oxide resistor as defined in claim 1, wherein each of said opposed zinc-oxide single crystals contains said manganese dissolved therein in the form of a solid solution, in an amount of 0.05 mol % or more with respect to zinc therein.
4. The zinc oxide resistor as defined in claim 1, wherein each of the opposed zinc-oxide single crystals has a length of 5 mm, a width of 5 mm, and a thickness of 0.5 mm; said bismuth-boron based oxide interface layer comprises, in oxide wt % equivalent, 37.0 to 22.7 wt % of  $B_2O_3$ , 3.8 to 1.9 wt % of  $Co_2O_3$  and 5.7 to 1.6 wt % of  $MnO_2$ , with the remainder being bismuth oxide.
5. The zinc oxide resistor as defined in claim 1, which exhibits an  $\alpha$ -value of 20 or more, as a performance index of a zinc oxide varistor.
6. The zinc oxide resistor as defined in claim 1, wherein said zinc oxide resistor has an operating voltage of  $2.9 \pm 0.3$  V, as a performance index of a zinc oxide varistor.
7. The zinc oxide resistor as defined in claim 1, wherein (n+1) of zinc-oxide single crystals and (n) of bismuth-boron based oxide interface layer are alternately stacked, where n is a natural number of 2 or more, and

## 14

wherein said zinc-oxide resistor has an operating voltage of  $(2.9 \pm 0.3) n$  V, as a performance index of a zinc oxide varistor.

8. The zinc oxide resistor as defined in claim 1, wherein said zinc oxide resistor has an operating voltage of x V, as a performance index of a zinc oxide varistor, wherein n of zinc oxide resistors are electrically connected in series, where n is a natural number of 2 or more, wherein said zinc-oxide resistor has an operation voltage of  $n \times x$  V, as a performance index of a zinc oxide varistor.

9. A method of producing the zinc oxide resistor as defined in claim 1, comprising:

disposing an oxide containing bismuth and boron, between a pair of opposed zinc-oxide single crystals to form a sandwich structure of (a zinc-oxide single crystal/a composition to be formed as a glass phase/a zinc-oxide single crystal);  
heating and holding said sandwich structure at a high temperature allowing said oxide containing bismuth and boron, to be molten; and  
rapidly cooling said heated sandwich structure to join said pair of zinc-oxide single crystals with a glass-phase oxide interface layer intervening therebetween.

10. The method as defined in claim 9, includes:  
bringing each of two zinc-oxide single crystals into contact with a chunk of oxide cobalt, and heating said zinc-oxide single crystals and said chunk of oxide cobalt at a high temperature capable of inducing a diffusion reaction to diffuse cobalt from said chunk of oxide cobalt into said zinc-oxide single crystals so as to prepare each of said opposed zinc-oxide single crystals in such a manner as to have a cobalt concentration of 0.5 mol % or more.

11. The method as defined in claim 9, wherein:  
each of the opposed zinc-oxide single crystals has a length of 5 mm, a width of 5 mm, and a thickness of 0.5 mm; said oxide containing a primary component consisting of bismuth and boron, to be used for forming a junction between said opposed zinc-oxide single crystals, is a glass prepared in such a manner as to contain, in oxide wt % equivalent, 37.0 to 22.7 wt % of  $B_2O_3$ , 3.8 to 1.9 wt % of  $Co_2O_3$  and 5.7 to 1.6 wt % of  $MnO_2$ , with the remainder being bismuth oxide.

12. The method as defined in claim 9, wherein said oxide containing a primary component consisting of bismuth and boron, to be used for forming a junction between said opposed zinc-oxide single crystals, is a glass, wherein said method includes:

flattening each surface of said opposed zinc-oxide single crystals through mirror polishing; and  
adjusting a quantity of said glass in such a manner that a molar ratio of said glass quantity in an equivalent bismuth quantity contained in said glass to a quantity of said opposed zinc-oxide single crystals, is set at 1.2 mol %.

\* \* \* \* \*